

(Model.)

T. S. GILBERT.

CORSET STAY.

No. 259,128.

Patented June 6, 1882.



Witnesses.

J. A. Shumway  
John Earle

Thomas S. Gilbert  
Inventor

By atty.

John Earle

# UNITED STATES PATENT OFFICE.

THOMAS S. GILBERT, OF NEW HAVEN, CONNECTICUT, ASSIGNOR TO MAX ADLER, OF SAME PLACE.

## CORSET-STAY.

SPECIFICATION forming part of Letters Patent No. 259,128, dated June 6, 1882.

Application filed December 12, 1881. (Model.)

*To all whom it may concern:*

Be it known that I, THOS. S. GILBERT, of New Haven, in the county of New Haven and State of Connecticut, have invented a new Improvement in Corset-Stays; and I do hereby declare the following, when taken in connection with the accompanying drawing and the letters of reference marked thereon, to be a full, clear, and exact description of the same, and which said drawing constitutes part of this specification, and represents a transverse section enlarged.

This invention relates to the construction of a substitute for bones in corsets.

It is well known that tampico-fiber has a certain amount of elasticity, and has been used in corsets as a substitute for whalebone and other stays.

Various devices have been resorted to to retain fiber in the proper shape for insertion into the corset, such as twisting the fiber into a cord, or by winding several fibers, or by an outside covering over several fibers, or clasps around several fibers to bind them together.

These constructions, however, are not only difficult but expensive to make.

The object of this invention is to combine several fibers into a single stay without such outside connections, attachment, or covering; and it consists in a corset-stay composed of several fibers of tampico or equivalent material running longitudinally of the stay, secured together by an adhesive material between the fibers, which serves as the means for securing the said longitudinal fibers together and without the intervention of transverse or other binding fiber or means. The best method known to me for thus combining several fibers to form a single stay is to take the number of fibers required for the production of a given size of stay, then, holding them together, draw them through a bath of india-rubber in solution, taking off the surplus as it

passes from the bath, and then vulcanizing the whole. This firmly secures the fibers together in their proper shape for insertion into the corset, the security being throughout their entire length and water-proof, so that the stay is not affected by the perspiration of the wearer.

Instead of drawing the fibers through the bath together, they may be immersed separately in the india-rubber, and connected after such immersion, the adhesive nature of the india-rubber holding them together, and presenting substantially the same stay as in the first instance.

Instead of india-rubber, gummy or adhesive material may be used for connecting the several fibers; but I prefer the india-rubber from its well-known adhesive and water-proof qualities.

While I prefer to combine the fibers into a stay so that the fibers lie parallel to each other, they may be twisted; but in either case the india-rubber, adhesive material, or gum serves to hold the several fibers together to complete the stay.

From the foregoing it will be understood that I do not broadly claim a stay made from fibers, as such, I am aware, is not new; but in all previous constructions of stays of this character some mechanical device has been required to be applied to hold the fibers in their proper relation to each other—that is, to secure them together to form the stay.

I claim—

A corset-stay composed of several fibers of tampico running longitudinally of the stay, secured together by india-rubber or adhesive material between the said fibers, substantially as described.

THOS. S. GILBERT.

Witnesses:

JOS. C. EARLE,  
LILLIAN D. ROGERS.